

# UNITED STATES PATENT OFFICE.

SAMUEL HEMAN THURSTON, OF LONG BRANCH, NEW JERSEY.

## PROCESS OF COATING ONE METAL WITH ANOTHER, &c.

SPECIFICATION forming part of Letters Patent No. 622,732, dated April 11, 1899.

Application filed July 2, 1898. Serial No. 685,073. (No specimens.)

*To all whom it may concern:*

Be it known that I, SAMUEL HEMAN THURSTON, a citizen of the United States of America, residing at Long Branch, county of Monmouth, State of New Jersey, have invented and made a certain new process for coating one metal with another, such as iron and steel with copper, and a new product as the result of such process; and I do hereby declare that the following is a full, clear, and exact description and specification of the same.

My invention relates to the coating of metals in general with another metal of a softer nature in order to protect it from oxidation, and, specifically, to coating iron and steel with copper film or pelmicle, and to the furnishing of a product having a surface coating practically permanent in its nature in regard to its appearance and power of resisting changes from contact with the atmosphere; and it consists in a certain method of procedure fully set forth in this specification and claimed at the end thereof.

In order that persons skilled in the art to which my invention appertains may understand, perform, and use my invention, I will proceed to describe it.

I am aware that it is old in the art to coat one metal with another for various purposes by electrical process, by dipping in molten metal, by dipping in hot solution, by rolling two metals together after soldering them, and by rubbing an alloy of metal on iron to give color; but I am not aware that one metal has ever before my invention been permanently secured to another metal by means of the process I am about to describe, nor has any product ever been known in any way similar to the product which is furnished by the practice of my invention or process or ever produced by any other means, whether by my process or not.

My invention is confined to coating iron and its derivatives with a film of copper oxid. I shall in this present specification particularly so describe the steps necessary for this purpose.

Having thoroughly cleaned the surfaces of the iron to be coated—by cleaning I mean purifying the surfaces from matter which prevents cohesion of the coating metal with the molecules of the iron—I rub the said surfaces with copper until a thin coherent film

adheres to the iron. This may best be done by light frictional impact oft repeated, as with revolving copper brushes, which causes the copper to impinge or be impacted against the iron molecules and into the interstices and to cohere with them. I then preferably heat the iron provided with the said copper film to a heat sufficient to turn the said film to a deep blue-black, and leave on the iron a thin skin of black oxid of copper or cupric oxid, which adheres so tenaciously to the iron as to practically form a part of the iron itself. I sometimes heat the iron before coating it to drive off any moisture there might be present. The cupric oxid formed is very dense and quite black and serves as a perfect protection for the iron against the atmospheric attacks. It is to be here stated that the copper film will adhere to the iron and protect its surfaces, even if it is not changed to a black cupric oxid, and for some especial purposes I propose to stop my process at this point. This copper film adheres so tenaciously to the iron as to resist removal by bending, rolling, or hammering, and can only be filed off or removed by abrasion. Coat after coat may be applied in the manner heretofore described until a thickness is attained suitable for the uses to which the product is to be put. This is particularly true when the cupric oxid is formed from the film, and a copper film may be formed over the cupric-oxid film and not again heated to form another coating of cupric oxid; but I prefer for most purposes to carry my process to its full limit and leave a film of cupric black anhydrous oxid of copper on the iron of such thickness as will be sufficient for the special purposes needed.

I am aware of the United States patents to Bower, January 2, 1883, and Spring, November 27, 1877; of English patents to Dowling, 1839, No. 7,949, and to Barron, May 24, 1856, No. 1,243, and I do not claim anything set out in said patents. By exhaustive experiments I have determined that the oxid of copper will not stick to copper, as their coefficient of expansion is different from the coefficient of expansion of copper, while the coefficient of expansion of copper oxid and that of iron correspond closely enough to prevent scaling off. I have applied copper in a comminuted form; but I prefer to comminute it by rubbing it on

the iron and at the same time force it into the pores of the metal.

Having now fully described my invention and the manner in which I have embodied it, 5 what I claim as new and as my invention, and desire to secure by Letters Patent, is—

1. The within-described process of coating iron and steel with copper oxid, which consists in first cleaning the iron to be coated and 10 then causing either metal to impinge upon the other metal until a film of copper is impacted upon the iron to be coated, and then

heating the said film to the desired temperature to form cupric oxid, substantially as and for the purposes hereinbefore specified.

2. The within-described product consisting of iron or steel covered with an adherent coating of oxid of copper, substantially such as hereinbefore specified.

SAMUEL HEMAN THURSTON.

Witnesses:

JAMES M. HICKS,  
CHARLES W. Low.